

# United States Patent Office

3,330,658

Patented July 11, 1967

1

3,330,658  
PHOTOGRAPHIC SILVER HALIDE DIFFUSION  
TRANSFER PROCESS

Paul B. Gilman, Jean E. Jones, and Arthur A. Rasch,  
Rochester, N.Y., assignors to Eastman Kodak Company,  
Rochester, N.Y., a corporation of New Jersey  
No Drawing. Filed Dec. 20, 1963, Ser. No. 332,305  
10 Claims. (Cl. 96—29)

### ABSTRACT OF THE DISCLOSURE

Silver images of improved tone are obtained in the silver halide diffusion transfer process by developing an exposed silver halide emulsion layer and transferring the silver halide from the undeveloped areas of the emulsion layer imagewise by diffusion to an image receiving layer containing physical development nuclei for dissolved silver salts, the transferring being effected with the emulsion layer and the image receiving layer in contact with a silver halide solvent and a dithiabiquaternary ammonium salt having the general formula



wherein  $R_1$ ,  $R_2$  and  $R_3$  each represent alkylene groups and  $Q$  and  $Q_1$  each represent a quaternary ammonium salt group selected from the class consisting of (1) trialkyl ammonium salt groups having the formula



in which the  $R$  groups are lower alkyl and  $X$  is an anion and (2) a salt group having the formula



in which  $Z$  represents the atoms necessary to complete a  $N$ -heterocyclic ring selected from the class consisting of pyridyl, piperidyl and morpholinyl,  $X$  is an anion and  $R_4$  is selected from the class consisting of hydrogen and lower alkyl.

This application is a continuation-in-part of U.S. application Ser. No. 141,036, filed Sept. 27, 1961.

This invention relates to photography and more particularly to a photographic diffusion transfer process in which silver images of improved tone are obtained.

In the well-known silver halide diffusion transfer process of photograph, an exposed emulsion layer is developed in the presence of a silver halide solvent, the emulsion layer being for at least a portion, or for the whole of the development period in effective contact with a receiving sheet, the surface of which generally carries a quantity of a silver precipitant which may comprise either physical development nuclei such as colloidal silver or silver sulfide or a chemical precipitant for silver ions, such as zinc sulfide. Development of the emulsion layer proceeds, and concurrently the residual unexposed silver halide is dissolved by a silver halide solvent also present in the developer composition, followed by imagewise diffusion of the resulting silver complex to the receiving sheet where the silver precipitant catalyzes physical development and causes the formation of an argental image. 65 groups e.g. methyl, ethyl, propyl, butyl etc. and  $X$  is an

2

In this process the argental image has a characteristic yellow, brownish or other unacceptable color whereas a neutral toned image is desired.

It is known to use toning agents to obtain a neutral tone. The toning agent is customarily added to the developer or to the receiving sheet so that when the silver image is formed, the silver grains are of sufficient size to provide a neutral or black image. However, many of the toning agents which are known for toning in the conventional chemical developing process, when used in the diffusion transfer process, result in positive images which do not have satisfactory gradation in contrast. For instance, these images would not be suitable for continuous tone reproduction, but only for office copying or similar uses where extreme contrast is desired.

In the Tregillus et al. U.S. Patent 3,017,270, for example, various tone modifying components are used in conjunction with quaternary ammonium salts with a linear chain of at least 7 atoms attached directly to a quaternary nitrogen atom. However, this combination acts on the silver halide emulsion to increase the development in the negative so that the resulting positive print, while it is of a neutral tone, may lack satisfactory gradation in contrast.

It has been desirable, therefore, to find an acceptable toner which would not only result in the neutral tone, but which would also provide the desirable gradation in contrast to provide suitable pictorial quality in the positive print. Suitable toners must also be compatible with a silver halide emulsion, must not have a detrimental effect on the speed of the system and must not be deleterious to the ease of processing.

Inasmuch as the toner must be present during the formation of the silver grains in the receiving sheet and is preferably incorporated in the developer solution, the toner must also be compatible with the components in the developer. The amount of toner incorporated in the silver halide emulsion must be sufficient so that an adequate quantity leaches out during the silver halide transfer to affect the silver grain size. Therefore, finding suitable toners has been considered unpredictable in the diffusion transfer field.

We have discovered that if this process is carried out in the presence of dithiabiquaternary ammonium salts the image has the desired neutral tone. The salts are useful when incorporated into either or both the developer solution and the nucleated receiving layer of the process. The salts are particularly effective to produce neutral toned images when used in conjunction with sulfur compounds such as described below.

The dithiabiquaternary ammonium salts have the general formula



wherein  $Q$  and  $Q_1$  represent a quaternary ammonium salt group such as (1) a trialkyl ammonium salt group having the formula



in which the  $R$  groups are the same or different alkyl groups e.g. methyl, ethyl, propyl, butyl etc. and  $X$  is an

## 3

anion or acid radical, or (2) a salt group having the formula



in which Z represents the atoms necessary to complete a pyridyl ring e.g. pyridyl,  $\alpha$ -picolyl etc., a piperidyl ring or a morpholinyl ring, and X is as above;  $\text{R}_3$ ,  $\text{R}_1$  and  $\text{R}_2$  each represent alkylene groups such as ethylene, propylene, butylene, pentylene, tetradecylene etc.

The following are examples of the salts useful in our invention and having the above general formula:

3,10 - dithiadodecane - 1,12-bis-(N-methylpiperidinium-p-toluene sulfonate) (M.P. 180-182° C.)



3,13 - dithiapentadecane-1,15-bis-(N-methylpiperidinium-p-toluene sulfonate) (waxy solid)

624-988-3,8 - dithiadecane - 1,10 - bis - (N-methylpiperidinium-p-toluene sulfonate) (M.P. 152-155° C.)

3,18 - dithiaeicosane - 1,20 - bis - (N-methylpiperidinium-p-toluene sulfonate) (yellow viscous syrup)

3,13 - dithiapentadecane - 1,15 - bis - (N-methylmorpholinium-p-toluene sulfonate) (viscous syrup)

3,14 - dithiahexadecane - 1,16 - bis - (N-methylmorpholinium-p-toluene sulfonate) (viscous syrup)

3,9 - dithiaundecane - 1,11 - bis-(N-methylmorpholinium-p-toluene sulfonate) (viscous syrup)

1,4 - bis - (8 - aza - 6 - oxa - 7 - oxo - 3 - thiadodecyl)-1,4-dimethyl-piperazinium-p-toluene sulfonate



3,10 - dithiadodecane-1,12-bis-(methyldiethylammonium-p-toluene sulfonate) (M.P. 124° C.)

624-987-7,13 - dithianonadecane - 1,19 - bis - (pyridinium-p-toluene sulfonate) (M.P. 130-132° C.)

7,13 - dithianonadecane - 1,19 - bis - (2 - picolinium-p-toluene sulfonate)

The C, H, N, and S analytical values found corresponded to compounds having the formulas indicated above.

The salts mentioned can be prepared by either Procedure A or Procedure B illustrated below.

## PROCEDURE A



## PROCEDURE B



## 4

1,4 - bis - (3 - thia - 8 - aza - 7 - oxo - 6 - oxa dodecyl)-1,4-dimethyl piperazinium di-p-toluene sulfonate.—To a cold solution of 9.2 g. of sodium in 500 ml. of methanol was added 41.2 g. 1,4-bis( $\beta$ -mercaptoproethyl) piperazine. To the cooled reaction mixture there was added with stirring 71.8 g. of  $\beta$ -chloroethyl-N-butylcarbamate. The reaction mixture was allowed to remain at room temperature overnight, after which time the methanol was removed at reduced pressure. The residue was mixed with 250 cc. water and the whole extracted with chloroform. The chloroform was distilled and the residue collected.

Analysis.—Calcd.: C, 52.7; H, 7.4; N, 6.5; S, 14.8. Found: C, 53.0; H, 6.0; N, 6.1; S, 15.0.

$\beta$ -Chloroethyl-N-butyl carbamate.—To 800 g. 2-chloroethanol, 991 g. n-butyl isocyanate was added dropwise. After addition was complete the reaction mixture was heated on a steam bath for 2 hours then distilled under vacuum. Product distilled at 850/62 mm. to give 1700 g. carbamate (95 percent of theory).

7,13 - dithianonadecane-1,19-bis-(pyridinium-p-toluene sulfonate).—To a stirred solution of 23 g. (1 g. atom) of sodium in 500 ml. of methanol, there was added with cooling 68 g. (0.5 mole) of 1,5 pentanedithiol. After the addition of 136.5 g. (1.0 mole) of hexamethylene chlorohydrin with cooling and stirring, the reaction mixture was allowed to remain at room temperature overnight. The residue was mixed with one liter of water and the whole extracted with chloroform. The chloroform extract was dried over magnesium sulfate and then the chloroform was removed under reduced pressure. The residue was recrystallized from acetone. Yield 130 g. (72 percent of theory, M.P. 67.5°).

A mixture of 30.2 g. (0.1 mole) of the above 7,13-dithia-1,19-bis nonadecanediol and 100 ml. pyridine was treated with 39.4 g. (0.23 mole) of p-toluene sulfonyl chloride. After one hour below 20° C., there was added 150 ml. concentrated hydrochloric acid in one liter of water. The oil was extracted with chloroform, washed with dilute acid, separated and dried over magnesium sulfate. Removal of the solvent at reduced pressure gave a light yellow viscous oil.

A solution of the oil was dissolved in excess pyridine, heated at the boiling point for 15 minutes, cooled and poured into cold ether. The solid was filtered, washed with ether, and dried.

It has been mentioned that the dithiobisquaternary ammonium salts are particularly effective to tone the silver images when used with mercaptan compounds. These compounds are characterized in some instances by having a beneficial effect upon tone, but do not give the best image tone (neutral) in the present process except in combination with the mentioned quaternary salts. As will be seen in the following examples one or more dithiobisquaternary ammonium salts can be used alone, or with one or more of the organic sulfur containing compounds such as the following:

- 5-amino-2-mercaptop-1,3,4-thiadiazole
- 1-methyl-2-mercaptopimidazole
- 4-aminomethyl-2-mercaptopimidazole
- 4-cyano-2,3-dioxo-5-thionopyrrolidine
- 1,10-bis-(morpholino)-1,10-dioxo-2,5,6,9-tetrathiadecane
- 1,4-bis-(2-mercaptoproethyl)-piperazine
- 3-mercaptopypyridine-N-oxide
- 5-bromo-6-methyl-1,3,3a,7-tetraazaindene-4-thiol
- 6-phenyl-1,3,3a,7-tetraazaindene-4-thiol
- 2-mercaptopbenzoxazazole
- 2-mercaptopbenzimidazazole

- 5,6-dichloro-1-ethyl-2-thiobenzimidazolone  
 S-thiobenzoylthioglycolic acid  
 2-hydroxy-1-mercaptopro-3-naphthoic acid  
 Oxazoline-2-thiol  
 4-phenylimino thiourazole  
 3-mercaptopro-8-thia-1,2,3a-triazacyclopent [α] indene  
 3-mercaptopro-5-methyl-1,2,4-triazole  
 3,4-diamino-5-mercaptopro-1,2,4-triazole  
 5-anilino-4-phenyl-1,2,4-triazole-3-thiol  
 5-ethyl-3-mercaptopro-4-phenyl-1,2,4-triazole  
 3-mercaptopro-4-phenyl-1,2,4-triazole  
 N,N'-bis-(4,4'-picolythiourea)  
 3-mercaptopro-1,2,3a-triazaindene  
 N-(N'-phenylthiocarbamido)-morpholine  
 Ethyl-p-(3-methyl-2-thioureido) benzoate  
 10,13-dithia-5,18-dithio-4,6,17,19-tetraazadocosane-1,22-bis diethylamine  
 1,3-bis(4-dimethylaminophenyl)-thioureadimethyl-iodide  
 1-(p-acetylphenyl)-3-butylthiourea  
 4,6-diphenyl-6H-1,3-thiazine-2-thiol  
 Thiocarbostyryl  
 4-mercaptopro-1,2,3-triazaanaphthalene  
 3-mercaptopro-1,2,4-triazole  
 1-methyl-1,2,3,6-tetrahydro-1,3,5-triazine-4-thiol  
 1-(p-carboxyphenyl)-5-mercaptopro-4-oxazolone



- 1-carbamyl-5-mercaptopro-4-oxazolone  
 1-(3-acetamidophenyl)-5-mercaptopro-4-oxazolone  
 5-mercaptopro-1-(x-sulfophenyl)tetrazole K salt  
 1-(4-carbomethoxyphenyl)-5-mercaptopro-4-oxazolone  
 1-phenyl-5-(trichloromethylidithio)-tetrazole  
 5-mercaptopro-1-methyltetrazole  
 1-m-carboxyphenyl-5-mercaptopro-4-oxazolone  
 3,5-di-imino-1,2,4-dithiazole



- 4-methyl-5-methylimino-1,2,4-dithiazolidine-3-thione HBr  
 2,4-dimethyl-1,2,4-thiodiazolidine-3,5-thione  
 Bis-(5-phenyl-1,3,4-thiadiazol-2-yl)disulfide dimetho-p-toluenesulfonate  
 5-acetamido-1,3,4-thiodiazole-2-thiol  
 3-amino-5-mercaptopro-1,2,4-triazole  
 3-β-formamidoethyl-5-mercaptopro-1,2,4-triazole  
 4-amino-5-mercaptopro-3-phenyl-1,2,4-triazole  
 Thiourazole  
 1-(4-sulfamoylphenyl)-3-mercaptopro-1,2,4-triazole  
 1,2,4-triazole-3,5-dithiol  
 5-methyloxazoline-2-thiol



- 3-β-carboxyethyl-2-thio-2,4-oxazolidinedione  
 5-acetamido-2-mercaptopro-thiazole  
 2-thiazolidinethione



- 5-imino-3,4,4-trimethylthiazolidine-2-thione  
 Rhodanine  
 4-carboxy-2-phenyl-thiazolidine

- 2-mercaptoprothiazole  
 Carboxymethyl-N-thiazol-2-yl-dithiocarbamate  
 Bis-2-thiazolyl-disulfide  
 3-(2,2,2-trichloro-1-hydroxyethyl)-2-thiazolidinethione  
 5 3-aminorhodanine  
 3-(o-tolyl)-rhodanine  
 3-ethylrhodanine  
 3,4,5-trimethyl-4-thiazoline-2-thione  
 1-thiocarbamyl-3-ethoxy-5-pyrazolone



- 15 1-hydroxyethyl-2-mercaptopro-4,5-dihydroimidazole



- 20 1-acetyl-2-thiohydantoin  
 1-β-hydroxyethyl-imidazolidine-2-thione  
 1,3-di-phenyl-2-thiohydantoin

- 25 4-amino-methyl-2-mercaptopro-imidazole  
 4,5-dihydro-1-(4,5-dihydroimidazol-2-yl)-2-mercaptoproimidazole

- 5-p-dimethylamino-benzal-2-thiohydantoin  
 1-acetyl-5-[4-(2-hydroxyethoxy)benzylidene]-2-thiohydantoin

- 30 1-benzoyl-2-thiohydantoin  
 2,2,5,5-tetramethyltetrahydrothioglyoxaline-4-thione  
 Ethylenethiocarbamate



- Thiocarbonyl-bis-(pyrrolidine)

- 40 Bis-(tetramethylene)-thiuram sulfide

- 4-cyano-2,3-dioxo-5-thionopyrrolidine

- 2-thiophenaldehyde-thiosemicarbazone

- 5-p-chlorophenyl-2-mercaptopro-1,3,4,4H-thiadiazine

- 5-hydroxy-3-mercaptopro-6-methyl-1,2,4-triaza-benzene

- 5,6-di-methyl-3-mercaptopro-1,2,4-triaza-benzene  
 45 3-mercaptopro-5-phenyl-1,2,4-triaza-benzene  
 5-(2-hydroxyethyl)-1,3-dimethylohexahydro-5-triazin-2-thione

- 5-(2-hydroxyethyl)-1,3-bispolyoxyhexahydro-s-triazin-2-thione

- 50 N-β-mercaptoproethylmorpholine  
 1,10-bis-(morpholino) 1,10-dioxo-2,5,6,9-tetrathiadecane



- β,β'-bis-morpholinoethyl-disulfide

- 2-mercaptopro-3-morpholinopropanol

- Bis-(3-oxapentamethylene-carbamyl-oxoethyl)-disulfide  
 60 Bis-(β,N-methylmorpholinium-methyl)-disulfide  
 diperchlorate

- 4-keto-2-mercaptopro-tetrahydro-1,3-thiazine



- 4-amino-2-mercaptopro-1,3-thiazine-(2-thiocytosine)



2,4-dithiolpyrimidine  
4-amino-6-hydroxypyrimidine-2-thiol



2-mercaptop-4,5,6-triamino-pyrimidine  
4,5-diamino-6-hydroxy-2-mercaptopurimidine  
Thiouracil  
5-methylthiouracil  
2-thio-barbituric acid  
4,5-diamino-2-mercaptopurimidine  
4,6-dimethyl-2-thio-2,3-dihydropyrimidine  
4,6-diamino-pyrimidine-2-thiol  
2,6-diamino-4-mercaptopurimidine  
5-aminomethylene-1-ethyl-2-thiobarbituric acid  
4-amino-5-carbethoxy-2-mercaptopurimidine  
3,4,5,6-tetrahydro-3-methyl-4-oxopyrimidine-2-thiol  
2-amino-4-mercaptop-6-methylpyrimidine  
1,4-bis-(2-mercaptopethyl)-piperazine  
Bis-[2-(N-methyl-3-azapentamethylenecarbamyloxy)-ethyl]-disulfide  
1-methylpiperazine-4-ethanethiol  
Methyl-5-thioctate



1-[pyridinium(chloride)acetyl]-4-phenylthiosemicarbazide  
γ-3-mercaptopropyl-N-methylpyridinium-p-toluenesulfonate  
1:1 pentamethylene-3-pyrid-2'-yl-thiourea



2-mercaptopuridine-N-oxide



1,6-bis-[methyl-(2-γ-pyridylethyl)-dithiocarbamato]-hexane-dimethoperchlorate  
2-mercaptopethyl-5-hydroxy-4-pyrone  
6-hydroxy-3-mercaptop-5-methyl-1,2,3a,4,7-pentazaindene  
7-hydroxy-5-mercaptop-1,2,3,4,6-pentazaindene  
6-hydroxy-3-mercaptop-4-methyl-1,2,3a,7-tetrazaindene  
4-hydroxy-6-methyl-1,2,3a,7-tetrazaindene-3-thiol  
4-hydroxy-2-mercaptopethyl-6-methyl-1,3,3a,7-tetra-zaindene  
2-carboxymethylmercaptop-4-oxo-5-methyl-6-thiono-4,5,6,7-tetrahydro-1-thia-3,5,7-triazaindene  
4-mercaptop-1-thia-3,5,7-triazaindene  
6-ethoxy-2-(β-carboxy-β-thiolpropionamido)-benzothiazole  
6-ethoxy-2-(β-carboxy-α-thiolpropionamido)-benzothiazole  
4-hydroxy-6-mercaptop-1,2,5,7-tetrazaindene  
6-mercaptopurine  
7-methyl-6-thiopurine



4-amino-6-mercaptop-1-methyl-2-methylmercaptop-1,3,5,7-tetrazaindene



4,7-dihydroxy-2-mercaptop-1-phenyl-1,3,,5,6-tetrazaindene  
4,7-dihydroxy-2-mercaptop-1,3,5,6-tetrazaindene  
1-mercaptop-3-iminoisoindole  
1-methyl-4-thioquinazoline  
4-carbethoxy-1,5-dithia-3-oxospiro[5.5]-hendacane



3-mercaptop-1,2,3a,8-tetrazacyclopent-[α]-indene  
3-mercaptop-1,2,3a-triaza-benz[e]-indene  
1-mercaptop-5-methyl-2,3,9b-triazabenzol-[e]-indene  
2-mercaptop-5-(3-pyridyl)-1,3,4-thiadiazole  
5-(3-oxindolylidene)-rhodanine



3,6-di-(1,2-dihydro-1-methyl-quinolin-2-yl-1dene)-1,2,4,5-tetrathia-cyclohexane



The use of the mentioned quaternary ammonium salts in the diffusion transfer processes of the invention is illustrated by the following examples:

#### Example 1

A silver halide emulsion layer was exposed to a subject in a conventional manner then treated with the following developing solution:

|    |                              |       |        |
|----|------------------------------|-------|--------|
| 50 | Sodium sulfite               | grams | 60.0   |
|    | Elon                         | do    | 2.6    |
|    | Trisodium phosphate          | do    | 50.0   |
|    | Hypo                         | do    | 12.0   |
| 55 | Hydroquinone                 | do    | 4.6    |
|    | 0.5% carboxymethyl cellulose | cc    | 1000.0 |

The emulsion layer was then squeegeed into contact with the receiving sheet described below, with a layer of the solution between, and allowed to remain in contact until the exposed silver halide had developed to a silver image and the residual undeveloped silver halide had transferred as a complex with the hypo to the receiving sheet, where positive silver containing image was formed. The emulsion layer was then stripped away from the sheet to reveal the silver image which has a neutral tone. In carrying out the process, the exposed emulsion layer may be wetted with the developer solution, and by passage over and between a series of rollers, brought into contact with the receiving sheet, and the resulting laminated sheet rolled up upon a roller until the transfer step is complete, after which the sheets are separated. Apparatus suitable for this procedure is described in the Vincent U.S. patent application Ser. No. 132,687, filed Aug. 21, 1961. Alternatively, both of the sheets may be wetted before lamination is effected.

## RECEIVING SHEET

Part 1.—To one liter of water at 40° C. were added 500 ml. of 1% gelatin solution and 9.5 ml. of 0.2 molar sodium sulfide.

Part 2.—To one liter of water at 40° C. were added 7 ml. of 0.4 molar nickelous nitrate.

Part 2 was added to Part 1 dropwise with stirring for 2 minutes and the remainder of Part 2 added over a period of about 2 minutes. 45 grams of dry gelatin were added followed by stirring at 40° C. for about 15 minutes to obtain a dispersion of nickel sulfide in gelatin. The above-mentioned dithiabisquaternary ammonium salts were each added to portions of the melted dispersion in amounts of the order of 0.7 gram per liter of the dispersion. Next, 0.1 gram per liter of 3-mercaptop-1,2,4-triazole and 0.05 gram per liter of 5-methyl oxazoline-2-thiol were added to each batch, after which the compositions were coated upon separate paper bases.

When each receiving sheet was employed in the process described, a neutral toned image was obtained whereas when a similar nickel sulfide receiving sheet not containing the mentioned salt was used, a brownish toned image was obtained.

The use of the dithiabisquaternary ammonium salts alone as toning agents is illustrated by the following examples:

## Example 2

A silver halide emulsion No. 895 was exposed and developed in the following developer solution in contact with a nickel sulfide sheet similar to that of Example 1.

H<sub>2</sub>O ml. 700  
2-aminoethanol-sulfur dioxide ml. 180  
1-phenyl-4,4-dimethyl-3-pyrazolidone g. 0.50  
Hydroquinone g. 5.50  
Sodium sulfite, anhydrous g. 144  
Water to 2000 ml.

To this developer solution were added varying amounts of the compound No. 624-987 [7,13-dithianonadecane-1,19-bis-(pyridinium-o-toluene-sulfonate)] of from 0 to 0.8 gram per liter. As a result, when about 0.4 to 0.8 gram per liter was present the best image tone was obtained on the sulfide sheet, whereas in absence of compound 624-987 a yellow image was obtained on the sheet.

## Example 3

A sensitive element similar to that described in Example 1 of the Yackel et al. U.S. patent application Ser. No. 586,705, filed May 23, 1956, now U.S. Patent 3,020,155, comprising a cellulose ether phthalate-silver halide emulsion coated upon a zinc sulfide nucleated receiving layer on a support, was exposed then developed at 80° F. in the following developer solution for 1 minute.

Water ml. 2900  
1-phenyl-4,4-dimethyl-3-pyrazolidone g. 1.0  
Hydroquinone g. 9.0  
Sodium sulfite, anhydrous g. 240  
Sodium carbonate, anhydrous g. 86.4  
Hypo g. 135  
Compound 624-987 g. 1.9  
Water to 3200 g.

After this the element was immersed in 68° F. water to remove the emulsion layer containing a negative image, leaving a neutral toned silver image in the nucleated layer, whereas when the same developer solution free of compound 624-987 was used the image was yellow toned.

## Example 4

In the manner of Example 1 an exposed silver halide emulsion was developed in contact with a nickel sulfide coated receiving sheet containing about 20 mg. per square

| Compound                                                                                      | Contrast | No. of 0.3 log E Steps |
|-----------------------------------------------------------------------------------------------|----------|------------------------|
| 7,13-dithianonadecane-1,19-bis-(pyridinium-p-toluene-sulfonate)                               | 1.20     | 6                      |
| 3,6,9,12,15,18,21,24-octoxahexacosane-1,26-bis-(5-ethyl-2-methylpyridinium methane-sulfonate) | 2.30     | 3                      |

Another comparison was made with 3,8-dithiadecane-1,10-bis-(N-methylpiperidinium-p-toluene-sulfonate) and with each of  $\alpha$ -dimethylthiocarbamatomethyl-N-methylpyridinium-p-toluene-sulfonate and 4,4,10,10-tetraoxy-4,

foot of compound 624-987 using the following developer solution:

Sodium sulfite g. 60  
Hypo g. 12  
Sodium carbonate g. 50  
Hydroquinone g. 4.6  
Elon g. 4.0  
0.5% carboxymethyl cellulose ml. 1000

pH=11.0

to 85 cc. of which had been added 1.0 cc. 1% methanol solution of 3-mercaptop-1,2,4-triazole and 0.5 cc. of a 1% methanol solution of 1-methyl-1,2,3,6-tetrahydro-1,3,5-triazine-4-thiol, with the result that the silver image obtained on the nucleated receiver sheet was neutral colored. It was found that varying amounts of 624-987 in the sheet gave neutral images.

When the dithiabisquaternary ammonium salts e.g. compound 624-987 are used in the nucleated reception layers as described above, good image tone is obtained with from about 0.5 to 25 mg. per square foot; the mercapto compound, when present, such as 3-mercaptop-1,2,4-triazole, is useful in a range of about 0.05 to 20 mg. per square foot, and with 1-methyl-1,2,3,6-tetrahydro-1,3,5-triazine-4-thiol, about 0.05-20 mg. per square foot.

## Example 5

A silver halide emulsion layer was exposed and processed in contact with a nickel sulfide layer as described in Example 1 using the following developer:

Sodium sulfite g. 23  
Potassium sulfite g. 23  
Elon g. 6  
35 Hypo g. 7.7  
Kodalk g. 46  
Hydroquinone g. 15  
15 M NH<sub>4</sub>OH ml. 10  
Surfactant ml. 3.5  
Water ml. 1000

to which 70 cc. of a 1% aqueous solution of compound 624-988 and 10 cc. of 1% 3-mercaptop-1,2,4-triazole had been added. The resulting print on the sulfide layer was neutral toned.

## Example 6

3,6,9,12,15,18,21,24-octoxahexacosane-1,26-bis-(5-ethyl-2-methylpyridinium) methane-sulfonate was added at 0.4 g./l. to a melted dispersion in place of the dithiabisquaternary ammonium salt, as in Example 1, and positive images were prepared by the diffusion transfer system in the same manner. When the positive images using the quaternary salt and 5-methyl oxazoline-2-thiol were compared with those using the dithiabisquaternary with the same toner combination in the receiving layer, a great difference in image scale was apparent. While both images were of neutral tone, only the receiving sheet incorporating the dithiabisquaternary compound had sufficient gradation in density between highlight and shadow to result in a satisfactory continuous tone print. The contrast of sensitometric strips prepared using both receivers is as follows:

| Compound                                                                                      | Contrast | No. of 0.3 log E Steps |
|-----------------------------------------------------------------------------------------------|----------|------------------------|
| 7,13-dithianonadecane-1,19-bis-(pyridinium-p-toluene-sulfonate)                               | 1.20     | 6                      |
| 3,6,9,12,15,18,21,24-octoxahexacosane-1,26-bis-(5-ethyl-2-methylpyridinium methane-sulfonate) | 2.30     | 3                      |

11

10 - dithiatridecane-1,13-bis-pyridinium perchlorate with the following results:

| Compound                                                                    | Contrast | No. of 0.3<br>log E Steps |
|-----------------------------------------------------------------------------|----------|---------------------------|
| $\alpha$ -Dimethylthiocarbamatomethyl-N-methylpyridinium-p-toluenesulfonate | 2.5      | 3                         |
| 4,4,10,10-tetraoxy-4,10-dithiatriadecane-1,13-bispyridinium perchlorate     | 3.8      | 2                         |
| 624-988 (Control)                                                           | 1.2      | 6                         |

The dithia bis compounds were uniquely effective in providing the type of environment required for formation of positive prints with a full tone gradation, as well as neutral image tones.

The development nuclei used in the reception elements of the invention are those physical development nuclei for dissolved silver salts well known in the art including colloidal heavy metals, e.g. colloidal silver and gold, colloidal metal sulfides, selenides and tellurides, e.g. lead sulfide, nickel sulfide, cadmium sulfide, silver sulfide, copper sulfide, zinc sulfide, mercury sulfide; metal proteinates, e.g. silver proteinates; compounds forming physical development nuclei with dissolved silver salts, e.g. sodium sulfide, colloidal sulfur, organic sulfur compounds such as thiourea, mercaptans and xanthates. 20 25

Reception layers containing development nuclei suitable for use in the invention can be prepared by the reduction of metal salts in the presence of a hydrophilic organic colloid such as gelatin. In a preferred method, a soluble salt of a noble metal such as silver nitrate, gold, platinum, or rhodium chloride, is dissolved in a solution containing 0.5-2.0 percent concentration of gelatin or other hydrophilic colloids such as cellulose ether phthalate, or methyl methacrylate-methacrylic acid copolymer. To this solution is added an excess of an alkali hydroxide, carbonate, borate, or phosphate to form a suspension of hydrous metal oxide in a solution having a pH preferably in the range of 9-11. Next a solution of a reducing agent is added in concentration sufficient to at least partially reduce the metal oxide. Reducing agents commonly known to the photographic art may be used such as hydroquinone, monomethyl-p-aminophenol, hydrazines, etc. However, a preferred preparation employs formaldehyde, which serves both to reduce the metal oxide and harden the coating made from this solution. In a typical procedure a dispersion of silver resulting from reaction of silver nitrate, sodium hydroxide and a dilute formaldehyde solution was added to a 10% gelatin solution and coated upon a white pigmented cellulose acetatae butyrate support. If desired, the coating can also contain the mentioned quaternary ammonium salts of the invention such as compound 624-987 above.

Nuclei, which may be present in combination with the quaternary salts and the organic sulfur-containing compounds, can be applied in a solution of a colloid vehicle such as gelatin to a suitable support such as paper or a subbed cellulose ester or synthetic polymer support as described in the examples.

The silver halide emulsions used in the process to provide the silver halide image transfer to the reception layers, is not especially critical and for example silver bromide, silver chloride, and silver bromoiodide emulsions can be used. Naturally some variation in tone of the final silver image can be expected with different emulsions but in general the quaternary ammonium salts, particularly in combination with one or more of the organic, sulfur containing compounds, are effective to improve image tone.

Variations can be made in the composition of the developing solution. For example, the developing agent particularly non-diffusing ones can be contained all or in part in the emulsion layer. The silver halide solvent such as ammonium and alkali metal thiosulfates amines e.g. 2-amino ethanol N-diethyl amino ethanol etc. may be pres-

12

ent in the developing solution or in the receiving layer it only being necessary that the solvent be present to dissolve the undeveloped silver halide forming a complex that will diffuse to the nucleated receiving layer.

Quaternary salts are known to be used as sensitizers when incorporated in the silver halide emulsion. Their action is considered to be that of acceleration in both chemical and physical development. In a diffusion transfer system, physical development in the negative is undesirable. Therefore, the use of quaternary salts would be expected to have a detrimental effect on the positive image due to the physical development occurring in the negative. In the physical development, which occurs in the diffusion transfer process, silver is obtained from the unexposed silver halide emulsion to form the image in the receiving sheet by depositing silver on the nuclei. However, the presence of a quaternary salt tends to promote physical development in the silver halide emulsion and cause the developed silver in the emulsion to act as nuclei for deposition of silver from the unexposed silver halide. This, therefore, reduces the amount of silver available from the unexposed silver halide and markedly reduces the effectiveness of the silver halide transfer to the receiving sheet.

The invention has been described in detail with particular reference to preferred embodiments thereof, but it will be understood that variations and modifications can be effected within the spirit and scope of the invention as described hereinabove and as defined in the appended claims.

We claim:

1. A process for preparing a silver image of improved tone in a silver halide diffusion transfer process which comprises developing an exposed silver halide emulsion layer, transferring the silver halide from the undeveloped areas of the emulsion layer imagewise by diffusion to an image receiving layer containing physical development nuclei for dissolved silver salts, the transferring being effected with the emulsion layer and the image receiving layer in contact with a silver halide solvent and a dithia-bisquaternary ammonium salt having the general formula:



wherein  $R_1$ ,  $R_2$ , and  $R_3$  each represent alkylene groups and  $Q$  and  $Q_1$  each represent a quaternary ammonium salt group selected from the class consisting of (1) trialkyl ammonium salt groups having the formula



in which the R groups are lower alkyl and X is an anion, and (2) a salt group having the formula



in which Z represents the atoms necessary to complete a N-heterocyclic ring selected from the class consisting of pyridyl, piperidyl and morpholinyl, X in an anion, and R<sub>4</sub> is selected from the class consisting of hydrogen and lower alkyl.

2. The process of claim 1 wherein the salt has the general formula



5 wherein Q and  $Q_1$  are trialkylammonium salt groups and  
R<sub>1</sub>, R<sub>2</sub>, and R<sub>3</sub> each represent alkylene groups.

3. The process of claim 1 wherein the quaternary ammonium salt has the general formula



0 wherein  $R_1$ ,  $R_2$  and  $R_3$  each represent alkylene groups and  $Q$  and  $Q_1$  are pyridinium salt groups having the formula



in which Z represents the atoms necessary to complete a pyridyl ring, R<sub>4</sub> is selected from the class consisting of hydrogen and lower alkyl and X is an anion.

4. The process of claim 1 wherein the designated ammonium salt is a member of the class consisting of

- 3,10-dithiadodecane-1,12-bis-(N-methylpiperidinium-p-toluene-sulfonate)  
 3,13-dithiapentadecane-1,15-bis-(N-methylpiperidinium-p-toluene-sulfonate)  
 3,8-dithiadecane-1,10-bis-(N-methylpiperidinium-p-toluene-sulfonate)  
 3,18-dithiaeicosane-1,20-bis-(N-methylpiperidinium-p-toluene-sulfonate)  
 3,13-dithiapentadecane-1,15-bis-(N-methylmorpholinium-p-toluene-sulfonate)  
 3,14-dithiahexadecane-1,16-bis-(N-methylmorpholinium-p-toluene-sulfonate)  
 3,9-dithiaundecane-1,11-bis-(N-methylmorpholinium-p-toluene-sulfonate)  
 1,4-bis-(8-aza-6-oxa-7-oxo-3-thiadodecyl)-1,4-dimethyl-piperazinium-p-toluene-sulfonate  
 3,10-dithiadodecane-1,12-bis-(methyldiethylammonium-p-toluene-sulfonate)  
 7,13-dithianonadecane-1,19-bis-(pyridinium-p-toluene-sulfonate) and  
 7,13-dithianonadecane-1,19-bis-(2-picolinium-p-toluene-sulfonate).
5. The process of claim 1 wherein the ammonium salt during the transfer of the silver halide to the receiving layer is in effective contact with at least one organic sulfur containing compound selected from the class consisting of
- 5-amino-2-mercaptop-1,3,4-thiadiazole  
 1-methyl-2-mercaptopimidazole  
 4-aminomethyl-2-mercaptopimidazole  
 4-cyano-2,3-dioxo-5-thionopyrrolidine  
 1,10-bis-(morpholino)-1,10-dioxo-2,5,6,9-tetrathiadecane  
 1,4-bis-(2-mercaptopethyl)-piperazine  
 3-mercaptopyridine-N-oxide  
 5-bromo-6-methyl-1,3,3a,7-tetrazaindene-4-thiol  
 6-phenyl-1,3,3a,7-tetrazaindene-4-thiol  
 2-mercaptopbenzoxazole  
 2-mercaptopbenzimidazole  
 5,6-dichloro-1-ethyl-2-thiobenzimidazolone  
 S-thiobenzoylthioglycolic acid  
 2-hydroxy-1-mercaptop-3-naphthoic acid  
 Oxazoline-2-thiol  
 4-phenylimino thiourazole  
 3-mercaptop-8-thia-1,2,3a-triazacyclopent-[ $\alpha$ ]-indene  
 3-mercaptop-5-methyl-1,2,4-triazole  
 3,4-diamino-5-mercaptop-1,2,4-triazole  
 5-anilino-4-phenyl-1,2,4-triazole-3-thiol  
 5-ethyl-3-mercaptop-4-phenyl-1,2,4-triazole  
 3-mercaptop-4-phenyl-1,2,4-triazole  
 N,N'-bis-(4,4'-picolylthiourea)  
 3-mercaptop-1,2,3a-triazaindene  
 N-(N'-phenylthiocarbamido)-morpholine  
 Ethyl-p-(3-methyl-2-thioureido)-benzoate  
 10,13-dithia-5,18-dithio-4,6,17,19-tetrazadocosane-1,22-bis-diethylamine  
 1,3-bis-(4-dimethylaminophenyl)-thioureadimethyl-iodide  
 1-(p-acetylphenyl)-3-butylthiourea  
 4,6-diphenyl-6H-1,3-thiazine-2-thiol  
 Thiocarbostyrl  
 4-mercaptop-1,2,3-triazanaphthalene  
 3-mercaptop-1,2,4-triazole  
 1-methyl-1,2,3,6-tetrahydro-1,3,5-triazine-4-thiol  
 1-(p-carboxyphenyl)-5-mercaptopotetrazole



5

- 10 1-carbamyl-5-mercaptopotetrazole  
 1-(3-acetamidophenyl)-5-mercaptopotetrazole  
 5-mercaptop-1-(x-sulfonylphenyl)-tetrazole-K salt  
 1-(4-carbomethoxyphenyl)-5-mercaptopotetrazole  
 1-phenyl-5-(trichloromethylidithio)-tetrazole  
 5-mercaptop-1-methyltetrazole  
 1-m-carboxyphenyl-5-mercaptopotetrazole  
 3,5-di-imino-1,2,4-dithiazole

20

- 25 4-methyl-5-methylimino-1,2,4-dithiazolidine-3-thione-HBr  
 2,4-dimethyl-1,2,4-thiodiazolidine-3,5-thione  
 Bis-(5-phenyl-1,3,4-thiadiazol-2-yl)-disulfide-dimetho-p-toluene-sulfonate  
 5-acetamido-1,3,4-thiodiazole-2-thiol  
 30 3-amino-5-mercaptop-1,2,4-triazole  
 3- $\beta$ -formamidoethyl-5-mercaptop-1,2,4-triazole  
 4-amino-5-mercaptop-3-phenyl-1,2,4-triazole  
 Thiourazole  
 1-(4-sulfamoylphenyl)-3-mercaptop-1,2,4-triazole  
 35 1,2,4-triazole-3,5-dithiol  
 5-methyloxazoline-2-thiol



40

- 3- $\beta$ -carboxyethyl-2-thio-2,4-oxazolidinedione  
 5-acetamido-2-mercaptop-thiazole  
 2-thiazolidinethione

45



- 5-imino-3,4,4-trimethylthiazolidine-2-thione  
 Rhodanine

- 50 4-carboxy-2-phenyl-thiazolidine  
 2-mercaptopthiazole  
 Carboxymethyl-N-thiazol-2-yl-dithiocarbamate  
 Bis-2-thiazolyl-disulfide  
 3-(2,2,2-trichloro-1-hydroxyethyl)-2-thiazolidinethione  
 55 3-aminorhodanine  
 3-(o-tolyl)-rhodanine  
 3-ethylrhodanine  
 3,4,5-trimethyl-4-thiazoline-2-thione  
 1-thiocarbamyl-3-ethoxy-5-pyrazolone

60



- 65 1-hydroxyethyl-2-mercaptop-4,5-dihydroimidazole

70

- 70 1-acetyl-2-thiohydantoin  
 1- $\beta$ -hydroxyethyl-imidazolidine-2-thione  
 75 1,3-diphenyl-2-thiohydantoin



15

4-aminomethyl-2-mercaptop-imidazole  
 4,5-dihydro-1-(4,5-dihydroimidazol-2-yl)-2-mercaptopimidazole  
 5-p-dimethylamino-benzal-2-thiohydantoin  
 1-acetyl-5-[4-(2-hydroxyethoxy)-benzylidene]-2-thiohydantoin  
 1-benzoyl-2-thiohydantoin  
 2,2,5,5-tetramethyltetrahydroglyoxaline-4-thione  
 Ethylenetrithiocarbamate



Thiocarbonyl-bis-(pyrrolidine)  
 Bis-(tetramethylene)-thiuram sulfide  
 4-cyano-2,3-dioxo-5-thionopyrrolidine  
 2-thiophenaldehyde-thiosemicarbazone  
 5-p-chlorophenyl-2-mercaptop-1,3,4,4H-thiadiazine  
 5-hydroxy-3-mercaptop-6-methyl-1,2,4-triaza-benzene  
 5,6-di-methyl-3-mercaptop-1,2,4-triaza-benzene  
 3-mercaptop-5-phenyl-1,2,4-triaza-benzene  
 5-(2-hydroxyethyl)-1,3-dimethylolhexahydro-5-triazin-2-thione  
 5-(2-hydroxyethyl)-1,3-bipolyolhexahydro-s-triazin-2-thione  
 N-β-mercaptopethylmorpholine  
 1,10-bis-(morpholino)-1,10-dioxo-2,5,6,9-tetrathiadecane



β,β'-bis-morpholinoethyl disulfide  
 2-mercaptop-3-morpholinopropanol  
 Bis-(3-oxapentamethylene carbamoyloxyethyl) disulfide  
 Bis-(β,N-methylmorpholiniummethyl) disulfide  
 diperchlorate  
 4-keto-2-mercaptop-tetrahydro-1,3-thiazine



4-amino-2-mercaptopurine-(2-thiouracil)



2,4-dithiolpyrimidine  
 4-amino-6-hydroxypyrimidine-2-thiol



2-mercaptop-4,5,6-triamino-pyrimidine  
 4,5-diamino-6-hydroxy-2-mercaptopurine  
 Thiouracil  
 5-methylthiouracil  
 2-thio-barbituric acid  
 4,5-diamino-2-mercaptopurine  
 4,6-dimethyl-2-thio-2,3-dihydropyrimidine  
 4,6-diamino-pyrimidine-2-thiol  
 2,6-diamino-4-mercaptop-pyrimidine  
 5-aminomethylene-1-ethyl-2-thiobarbituric acid  
 4-amino-5-carbethoxy-2-mercaptop-pyrimidine  
 3,4,5,6-tetrahydro-3-methyl-4-oxopyrimidine-2-thiol  
 2-amino-4-mercaptop-6-methylpyrimidine  
 1,4-bis-(2-mercaptopethyl)-piperazine  
 Bis-[2-(N-methyl-3-azapentamethylene carbamoyloxy)-ethyl]-disulfide

16

1-methylpiperazine-4-ethanethiol  
 Methyl-5-thioctate



5  
 1-[pyridinium(chloride)acetyl]-4-phenylthiosemicarbazide  
 γ-3-mercaptopropyl-N-methylpyridinium-p-toluenesulfonate  
 10 1:1 pentamethylene-3-pyrid-2'-yl-thiourea



2-mercaptopurine-N-oxide



25  
 1,6-bis-[methyl-(2-γ-pyridethyl)-dithiocarbamato]-hexane-dimethoperchlorate  
 2-mercaptopethyl-5-hydroxy-4-pyrone  
 30 6-hydroxy-3-mercaptop-5-methyl-1,2,3a,4,7-pentazaindene  
 7-hydroxy-5-mercaptop-1,2,3,4,6-pentazaindene  
 6-hydroxy-3-mercaptop-4-methyl-1,2,3a,7-tetrazaindene  
 4-hydroxy-6-methyl-1,2,3a,7-tetrazaindene-3-thiol  
 4-hydroxy-2-mercaptopethyl-6-methyl-1,3,3a,7-tetrazaindene  
 35 2-carboxymethylmercaptop-4-oxo-5-methyl-6-thiono-4,5,6,7-tetrahydro-1-thia-3,5,7-triazaindene  
 4-mercaptop-1-thia-3,5,7-triazaindene  
 6-ethoxy-2-(β-carboxy-β-thiolpropionamido)-6-ethoxy-2-(β-carboxy-α-thiolpropionamido)-benzothiazole  
 40 6-ethoxy-2-(β-carboxy-α-thiolpropionamido)-benzothiazole  
 4-hydroxy-6-mercaptop-1,2,5,7-tetrazaindene  
 6-mercaptopurine  
 7-methyl-6-thiopurine



45  
 50  
 4-amino-6-mercaptop-1-methyl-2-methylmercaptop-1,3,5,7-tetrazaindene



55  
 60  
 4,7-dihydroxy-2-mercaptop-1-phenyl-1,3,5,6-tetrazaindene  
 4,7-dihydroxy-2-mercaptop-1,3,5,6-tetrazaindene  
 1-mercaptop-3-iminoisoindole  
 65 1-methyl-4-thioquinazoline  
 4-carbethoxy-1,5-dithia-3-oxospiro-[5·5]-hendecane



70  
 75  
 3-mercaptop-1,2,3a,8-tetrazacyclopent-[α]-indene  
 3-mercaptop-1,2,3a-triaza-benzo[e]-indene  
 1-mercaptop-5-methyl-2,3,9b-triazabenzol[e]-indene

17

2-mercaptop-5-(3-pyridyl)-1,3,4-thiadiazole  
5-(3-oxindolyidene)-rhodanine



3,6-di-(1,2-dihydro-1-methyl-quinolin-2-yl-iden)-1,2,4,5-tetrathia-cyclohexane



6. The process of claim 1 wherein the ammonium salt is 3,8 - dithiadecane - 1,10-bis-(N-methylpiperidinium)-p-toluene sulfonate and a member of the class consisting of 3-mercaptop-1,2,4-triazole and 1-methyl-1,2,3,6-tetrahydro-1,3,5-triazine-4-thiol is in effective contact with the silver halide during the transfer step.

7. A reception element adapted to receive a dissolved silver halide image diffusing thereto from a developed silver halide emulsion layer to form a silver image from the dissolved silver halide, comprising a layer containing a mixture of physical development nuclei for dissolved silver salts, in a compound having the general formula



wherein  $R_1$ ,  $R_2$ , and  $R_3$  each represent alkylene groups, and  $Q$  having  $Q_1$  each represents a quaternary ammonium salt group selected from the class consisting of (1) trialkyl ammonium salt groups having the formula



in which the  $R$  groups are lower alkyl,  $X$  is an anion, and (2) a salt group having the formula



18

in which  $Z$  represents the atoms necessary to complete a N-heterocyclic ring selected from the class consisting of pyridyl, piperidyl and morpholinyl,  $X$  is an anion, and  $R_4$  is selected from the class consisting of hydrogen and lower alkyl.

8. An alkaline photographic silver halide developing solution comprises a silver halide developing agent and a compound having the general formula



wherein  $R_1$ ,  $R_2$ , and  $R_3$  each represent alkylene groups, and  $Q$  and  $Q_1$  each represents a quaternary ammonium salt group selected from the class consisting of (1) trialkyl ammonium salt groups having the formula



20 in which the  $R$  groups are lower alkyl and  $X$  is an anion, and (2) a salt group having the formula



25 in which  $Z$  represents the atoms necessary to complete a N-heterocyclic ring selected from the class consisting of pyridyl, piperidyl and morpholinyl,  $X$  is an anion, and  $R_4$  is selected from the class consisting of hydrogen and lower alkyl.

9. The process of claim 1 wherein the physical development nuclei comprise nickel sulfide.

10. The element of claim 5 wherein the physical development nuclei comprise nickel sulfide.

35

#### References Cited

#### UNITED STATES PATENTS

|           |        |                  |       |           |
|-----------|--------|------------------|-------|-----------|
| 2,288,226 | 5/1942 | Carroll et al.   | ----- | 96-107 X  |
| 3,017,270 | 1/1962 | Tregillus et al. | ----- | 96-66.3 X |

NORMAN G. TORCHIN, Primary Examiner.

R. E. MARTIN, Assistant Examiner.